

Patented Dec. 22, 1925.

1,566,766

# UNITED STATES PATENT OFFICE.

GEORGE COLEMAN NIXON, OF SYRACUSE, NEW YORK.

## CASEHARDENING MATERIAL.

No Drawing.

Application filed October 20, 1923. Serial No. 669,736.

To all whom it may concern:

Be it known that I, GEORGE COLEMAN NIXON, a citizen of the United States, and a resident of Syracuse, county of Onondaga, 5 and State of New York, have invented a certain new and useful Casehardening Material; and I do hereby declare that the following is a full, clear, and exact description thereof, reference being had to the accompanying drawings, in which like numerals 10 refer to like parts.

This invention relates to an improved compound or material for use in casehardening iron or steel. Heretofore casehardening material has been made by adding to a suitable carbonaceous material, such as charcoal, coke, and the like, an energizer, such as 15 soda ash, lime, barium carbonate and the like.

What I claim as new and an improvement in the art is the use of an alkali metal phosphate, such as sodium phosphate or potassium phosphate, as an energizer in such compounds, either singly or in conjunction with 20 carbonates. By "phosphate" I mean either mono-phosphate or multi-phosphate, such as di- or tri-phosphate, all of which have a similar action.

One method of making the compound is to soak the carbonaceous materials, such as charcoal, coke, and the like, in a solution of alkali metal phosphate, such as sodium or potassium phosphate, until thoroughly saturated and then dry to make the finished 25 casehardening compound. One to ten percent, by weight, of said phosphate is desirable, although I do not limit myself to these proportions.

This casehardening material is peculiarly 30 well adapted for use in the dry packing process of casehardening and it will produce a deeper and an apparently harder case than similar compounds using soda ash, lime, barium carbonate and other old kind of energizer. Sodium or potassium phosphate has 35 never been known as an energizer, nor does it make carbon monoxide like the compound of carbonaceous material and soda ash and like old energizers. But how or why the phosphate energizes the carbonaceous material 40 for casehardening purposes, is not fully

known, nor what gas does result from said compound.

It is known, however, from careful and thorough tests, that it makes a thicker and 55 a harder case than a similar quantity of casehardening material heretofore known in the art and with similar use. The increase in the thickness of the case and in the hardness of the case is of very great importance in 60 the present highly developed state of the iron and steel art and especially in the automobile and aeroplane arts. Sodium and potassium phosphates are very soluble in 65 water and, therefore, are easy to mix with and impregnate the carbonaceous material.

By "carbonaceous material" herein is meant charcoal, coke or any other material containing considerable carbon, either 70 charred or uncharred, and adaptable for use in making compounds for casehardening iron and steel. By "energizer" herein is meant any chemical which is capable of rendering the carbonaceous material more active and effective in case hardening iron or 75 steel, such as barium carbonate, soda ash, lime, or other old energizers, as well as the new energizer herein set forth. By "alkali metal phosphate" herein is meant sodium or potassium phosphate, whether mono- or 80 multi-phosphates.

The invention claimed is:

1. Casehardening material including carbonaceous material, and an alkali metal phosphate mixed therewith. 85

2. Casehardening material including carbonaceous material, and sodium phosphate mixed therewith.

3. Casehardening material including carbonaceous material, and from one to ten 90 percent of an alkali metal phosphate mixed therewith.

4. Casehardening material including carbonaceous material, and from one to ten percent of sodium phosphate mixed therewith. 95

5. Casehardening material including carbonaceous material, and a multi-alkali metal phosphate mixed therewith.

6. Casehardening material including carbonaceous material, and tri-sodium phosphate mixed therewith. 100

7. Casehardening material including car-

- bonaceous material, and from one to ten percent of a multi-alkali metal phosphate mixed therewith.
8. Casehardening material including carbonaceous material, and from one to ten percent of tri-sodium phosphate mixed therewith.
9. Casehardening material including carbonaceous material impregnated with an alkali metal phosphate.

10. Casehardening material including carbonaceous material impregnated with a multi-alkali metal phosphate.

11. Casehardening material including carbonaceous material impregnated with tri-<sup>15</sup> sodium phosphate.

In witness whereof, I have hereunto affixed my signature.

GEORGE COLEMAN NIXON.